

W. D. HALL.

## PROCESS OF CASTING FROM VOLATILIZABLE METALS OR ALLOYS.

APPLICATION FILED JULY 9, 1913

1,100,132.

Patented June 16, 1914.

2 SHEETS OF PAPER



Witnesses:  
John E. Titus  
W. P. Kilroy

34 Inventor,  
By C. William D. Hall  
Luther Johns, Secy.

W. D. HALL.

## PROCESS OF CASTING FROM VOLATILIZABLE METALS OR ALLOYS.

APPLICATION FILED JULY 21 1963

1,100,132.

Patented June 16, 1914.

3 SHEETS-SHEET 2.



Fig. 9



Witnesses:  
John E. Tilus  
W. P. Kilroy

31 Inventor.  
William D. Hall  
By Luther Johns Mfg.

# UNITED STATES PATENT OFFICE.

WILLIAM D. HALL, OF OAK PARK, ILLINOIS.

## PROCESS OF CASTING FROM VOLATILIZABLE METALS OR ALLOYS.

1,100,132.

Specification of Letters Patent. Patented June 16, 1914.

Application filed July 9, 1913. Serial No. 778,006.

*To all whom it may concern:*

Be it known that I, WILLIAM D. HALL, a citizen of the United States, residing at the village of Oak Park, in the county of Cook and State of Illinois, have discovered a certain new and useful art and have invented a new and useful process and new and useful manufactures and certain apparatus for practising said process and art, of which the following is a description. In the present specification I have drawn claims to one branch of these discoveries and inventions — namely, the process of casting from volatilizable metals or alloys in impermeable refractory molds, such, for instance, as iron chills—but without abandoning other subject-matter herein disclosed.

A typical alloy of volatilizing properties, and one by which may well be illustrated the features of discovery and invention herein set forth, is brass, and by brass, as used in this specification, is meant an alloy the principal constituents of which by weight are copper and zinc. Yellow brass used for tubing and the like is usually a binary alloy composed of copper and zinc in the proportions, roughly speaking, of two to one in the order named, and practically all of the commercial brasses will be found to contain from 72% to 58% of copper and from 28% to 42% of zinc. Sometimes one or two per cent. of tin is added and sometimes a small proportion of aluminum, as in making the so-called "aluminum brass." Zinc, as is well known, is highly volatilizable. Indeed, it frequently happens in the making of brass that a cake of zinc lying on top of the molten copper in a crucible will suddenly volatilize in a flash—go up in smoke—and be totally lost. This tendency of the zinc to evaporation has been one of the main sources of difficulty in handling molten brass and has been prohibitive of any practical results in the casting of brass in refractory impermeable molds such, for instance, as iron chills having inclosed casting chambers. So great has been the demand for this art, however, that the problem has been essayed by metallurgists and mechanics persistently since beyond the memory of man, yet so inscrutable has appeared the solution in the past that after repeated failures and the loss of life many persons have come to regard this problem on a par with perpetual motion and have ridiculed my repeated efforts attended for years by repeated fail-

ures. An exemplification of the practice of this art by me, and one well suited to the purposes of this disclosure, is in the cast connections between various parts of a metallic bedstead. It is old to make iron connections cast in chills for bedstead frames. Where the bed frame parts to be connected are of iron, a cast iron connection is of course suitable, but where, as in many cases the bed frame is of brass rods or tubing or brass covered iron tubing the iron connection is not appropriate. In some such cases where the iron chill connections are used on brass rods the iron connection is bronze painted and lacquered to imitate brass; but this practice is obviously very unsatisfactory, as wear and the weather soon disclose the deception. This difficulty has been partly avoided in the past by making in sand brass castings of such shape as to fit upon the brass rods to be connected, then filing, dressing and polishing the brass castings, boring holes in them and also in the end portions of the rods and riveting or bolting the connection upon the parts to be held together. This method has various objections among which may be mentioned the time and labor involved in making the castings in the sand, the necessary fitting of the casting upon the parts, the filing, grinding or other means employed for dressing the casting to shape and finish, the cleaning and polishing, the boring of the holes and the riveting; and after all is thus done, at great expense, the connection is not as rigid as it should be, works loose and rattles, and is not in accordance with the best conceptions of the art, either mechanically or as to artistic effect.

The principal objects of this new art and of the invention or inventions by which it is practiced are to provide, by means of refractory impermeable molds, for instance iron chills having inclosed casting chambers, strong and sound castings from volatilizable metals and alloys, for instance the commercial brasses, and, as a notable departure, castings which are free from blow holes and other defects due to gases within the mold.

In specific applications the objects are to unite by mechanically perfect castings made from molten volatilizable metals or alloys poured into impermeable refractory molds rods, tubes or other structures of iron, brass, or other metals, and also to secure directly

upon such structures, sound and perfect castings of volatilizable metals or alloys.

In still more specific applications the objects are to secure or unite together brass or other rods, such as are employed in bedstead frames, by means of molten brass poured into an iron chill or other refractory impermeable mold, and generally to overcome thereby the disadvantages of the present methods of uniting such parts; to save much of the time, labor and other expense incident to the process now employed in making brass castings and in connecting such parts; to provide a strong and serviceable connection between such parts and one which will not work loose; to provide a connection of the same kind and color of material as that of the brass bedstead parts so connected; to form connections of the kind mentioned *in situ* upon the parts; to make such castings quickly and repeatedly from the same mold; to provide castings of the character mentioned which are free from blow holes, unfilled portions and the like defects; to provide such castings wherein the lines and marks of ornamentation are clear cut, and in which the casting is clean and smooth and requires little or no further work or polishing.

30 Still other objects will appear hereinafter. In the accompanying drawings, which form a part of this specification, I have shown as illustrative of means and results in the practice of the art herein described certain devices as employed and made by me in the bedstead making art.

In these drawings Figure 1 is a face view in open position of a two-part mold with tubes positioned therein ready to be secured together by molten metal. Fig. 2 is a top view of the parts shown in Fig. 1, the two halves of the mold being brought together ready for pouring and locked. Fig. 3 is a central vertical section through the mold shown in Fig. 1 with the mold closed, the tubes to be connected being shown in full. Fig. 4 shows fragmentary transverse sections on the line 4-4 of Fig. 1, the fragments being brought together. Fig. 5 shows fragmentary transverse sections on the lines 5-5 of Fig. 1, the fragments being brought together. Fig. 6 shows the two rods of Fig. 1 as connected by a casting made in the mold of Fig. 1. Fig. 7 is an elevation of a bedstead end frame, its parts being connected in the manner herein set forth and showing also ornaments formed directly upon the parts. Fig. 8 is a face view of a two-part mold in open position adapted to the casting of a knob upon a rod. Fig. 9 is a fragmentary vertical section, after a pour has been made, on the line 9-9 of Fig. 8, the mold sections being brought together, the casting and the rod being shown in full.

65 In the practice of this art by me iron

chills are employed, but any suitable refractory and impermeable material such as, it is thought, fire clay or composition may be used if found desirable enough. The word "mold" or "chill" as used in this specification is intended to distinguish from molds made of sand and the like permeable materials and which are formed anew for each individual casting, and also from iron molds in which a material portion or portions thereof are filled or lined with sand or equivalent permeable material placed therein for the purpose of permitting air or gas within the mold to filter through or permeate the sand and thus escape from the casting chamber, this distinction being intended to point out more definitely the domain of the present art as outside of that realm in casting processes wherein the seepage or filtering through or permeation of sand or equivalent substances by air or gas within the mold is vital and essential to the practice. This distinction from chills having a metallic portion thereof lined or filled with sand does not necessarily exclude from this art the casting of brass or other volatilizable metal or alloy in chills in which a sand core is employed for providing a hollow interior to the casting, as in the casting, for instance, of faucets or other types of valves and similar articles, and in which it may be found expedient to permit an end or the ends of the core to extend through the mold or in communication with an opening leading to the exterior of the mold. In some casting operations it may be desirable to give escape to the expanding air within the core itself, when the hot metal contacts the core, in order to prevent disintegration of the core by reason of the interior force of the expanding air. Where I employ cores, as indicated, I sometimes vent the core for the purpose stated; but the casting is made according to the present process and the casting chamber is freed of the gases of volatilization therein by means which do not depend upon the permeability of the core whatsoever. It is also pointed out that the practice of this art contemplates a chill or mold in which the casting chamber of the mold is surrounded or substantially surrounded by the walls thereof, and must be reached by a pouring duct leading from the outside of the mold. This distinction is made in order to negative any supposition that the present art is intended to include the mere pouring of volatilizing molten brass or other volatilizable metal or alloy into what is essentially an open hole or recess in iron, as, for instance, a mold of the character illustrated by the pour or vent channels shown in the drawings, should their respective openings into the casting chamber be closed. I wish also to distinguish the brass and other volatilizable

metals or alloys referred to in the description and in the claims from alloys which are sometimes called "brass," but which do not come within my hereinabove definition, 5 and also from metals or alloys which may to some extent have a volatilizable element, but not in sufficient proportions to make their casting in sandless chills a serious or any question. Thus, journal bearing alloys 10 are frequently called "brass," and disclosures have been made of molds in which the terms "car brasses," "engine brasses," etc., are used, when, as is well known, the alloy employed for such bearings is not brass at all, but bronze, and consists, roughly speaking, of nine parts of copper to one part of tin. Such so-called "brasses" and their casting in chills, therefore, are outside of the domain of the present disclosure, and 15 never have presented any difficulty of the character herein set forth. Sometimes, indeed, a small percentage (say from 1% to 4%) of zinc has been added to such "brasses," but rarely, inasmuch as even so 20 small an amount of zinc in journal bearings is bad practice, the zinc crystallizing in service and badly cutting and heating the journal. I am not aware, however, that it has ever been successfully attempted to cast 25 such so-called "brasses" in sandless molds where the alloy contained even a small percentage of zinc, as indicated, but understand that heretofore wherever there have been small or large quantities of gas to contend 30 with, molds partly or entirely of sand have been employed. Such bearing metals may 35 be cast in chills as herein set forth. I may mention, also, that there is an alloy called "acid brass" consisting of copper, tin, lead 40 and antimony, which, obviously, is not a brass. On the other hand, so-called "manganese bronze" consisting, according to one 45 formula, of 63 1/4 copper, 42% zinc, 3.75% manganese and 1.25% lead, clearly falls 50 within the class of volatilizable alloys which may be cast in chills according to the present teaching. The nomenclature of these yellowish alloys is not, therefore, always to be depended upon; but from the foregoing 55 it will be appreciated, and I desire it so to be understood, that my present discoveries and inventions are primarily in a domain of the art of casting where the gases of volatilization given off during the casting process are of considerable quantity; and it may 60 be generalized that the to me known domain of these discoveries and inventions is in the casting of the commercial brasses, as herein specified, and other metals or alloys which 65 give off at their casting temperatures substantially the quantities of fumes, vapors, or gases of volatilization as are produced by the commercial brasses, as hereinabove referred to, at the casting temperature herein set forth. The appended claims should 70 be construed therefore as including in their scope the commercial brasses as herein specified, and be given such additional scope as the nature of these discoveries and inventions, their utility, and their novelty in view of any prior practices may entitle them to. 75

It is here pointed out that the sudden chilling function of the iron mold as usually employed for iron is designedly omitted from the practice of the art herein set forth. It will be observed that the mold or chill 80 is much larger proportionately than the chill used for casting the same kind and size of connections from iron, and I preferably make my molds for this art about five times as large and heavy as for pouring iron. This additional size and weight are provided not only for the sake of safety, but, very importantly, in order to secure the retention 85 of a high degree of heat in the mold. 90

Whenever brass is melted a considerable quantity of the zinc which it contains is lost through volatilization, and, if not carefully melted, this loss may be as high as 10% in ordinary practice. The vapor of volatilization coming into contact with the air burns, forming oxide of zinc. For casting brass in chills the metal must be brought to a high temperature and must be poured quite hot. In this practice the molten brass is at a 95 bright red heat, verging on white heat, and consequently the fumes and gases given off are of great volume. At the desired heat the fumes of the zinc burn with an intensely 100 bright greenish tinted flame. The great problem has been to free the inclosed casting chamber of these gases and fumes. Thus far it has been impossible to introduce sufficient of such metal or alloy into 105 the chill to produce a casting free from blow holes or other large unfilled areas. A succession of vent recesses between the two valves of the chill as close to each other as it is possible to make them is ineffective, and 110 without the many unsatisfactory devices which I designed and tested for the purpose indicated was an elaborate system of suction by means of a vacuum chamber connected by a large number of ducts to the interior of the mold. 115

Referring to the drawings it will be seen that for the purpose of casting the forms there shown only two openings are provided leading to the interior or casting chamber of the mold. These are both in the form of channels having a considerable area at the top and gradually tapering to a smaller area where they join the hollow interior. These channels may conveniently be of complementary trough-like recesses as in Fig. 1. In all of the figures 21 is the pouring channel and is given preferably a circular mouth of relatively large area and the channel has a large capacity for pouring. This 120 125 130 135

channel may be suitably curved, and is preferably so directed that the pouring metal will discharge somewhat against the rods inserted within the mold, and this to prevent the constant discharge of the highly heated metal against the wall of the mold. In the preferred construction illustrated this pouring channel 21 preserves its substantially circular cross area from the top to the bottom and opens into the casting chamber 23 with an orifice of considerably larger cross area than is necessary for the pouring of iron, to wit, about five times such area. This pouring channel 21 enters the chamber 23 preferably at or very near its highest point when in casting position, in the patterns illustrated, to avoid pocketing of air and gas. The mouth of the channel 21 opens preferably into a transverse channel formed by the upright portions or walls 24 and 25 of the mold whereby the waste or overflow discharge of molten metal during the pouring operation will be conveyed to the sides of the mold where such metal may fall upon the ground without striking and injuring the rod 27 protruding from the mold. The upright portion 25 is designed also to protect the vertical rod 26 from the splashing of the molten metal while it is being poured. The pouring channel is preferably made on curved lines to provide greater capacity, as shown in Fig. 1. The vent channel 22 is preferably substantially circular in cross area where it enters the casting chamber 23, and of substantially the same area at this point as that of the discharge orifice of the pouring channel 21, as indicated in Figs. 4 and 5. The vent channel preferably gradually enlarges in cross area upward and outward. The outer discharge opening may be conveniently formed somewhat elliptical instead of circular, and it is not conceived that the exact shape of the vent channel is controlling, although its capacity and arrangement are vital. The vent channel may be curved in such manner, as in Fig. 1, that the gases will be reflected outwardly, but it may be on straight lines as in Fig. 8. The vent channel 22 enters the casting chamber 23 at or substantially at the highest point thereof when the mold is in casting position, as shown in the drawings.

The parts to be connected by the molten metal are shown in Fig. 1 in the form of two tubes 26 and 27 positioned at right angles to each other in the mold. The tube 26 is preferably provided with a closure, suitably in the form of a metallic cap 28 which frictionally fits over the end of the tube and is adapted to prevent the molten metal from filling a portion of the tube and thus being wasted. The tube 27 is shown as passing through the mold, each half of the mold having complementary recesses as at 26<sup>a</sup> and 27<sup>a</sup> for the accommodation of these pipes, as

is well understood in the old art of casting iron in chills. The two sections of the chill are suitably hinged together as by lugs 29 on one section and lug 30 on the other section connected by the hinge pin 31. Preferably on the edge portion of the mold opposite the hinge means are provided for clamping the two sections together for pouring, these means comprising in a simple form a bolt 32 threaded into the enlarged portion 33 of one section of the mold and having the turned portion or head 34 adapted to engage the outer face of the other chill section, as well illustrated in Figs. 2 and 8. It is here explained that before good and uniform results can be obtained the mold must be brought to a fairly high temperature, which may be done in the first instance by filling it several times with molten metal—preferably iron if conveniently to be had—for it is not desirable in the practice of this art that the brass castings cool as rapidly as iron castings or as rapidly as they would cool in chills which have not been well heated beforehand. Furthermore, it is necessary to have the mold quite hot in order that the molten brass will run freely into it and not chill unduly before the mold is completely filled. If castings are being continuously made, the successive pourings after the first may be made without taking this preliminary step of heating the mold. The mold having been sufficiently heated and tightened together with the parts to be connected positioned within the mold, the pouring may be made. The brass having been melted—say in a crucible—a sufficient quantity at the heat indicated is preferably transferred to a pouring ladle and skimmed, and the metal is then quickly emptied into the mold. The pouring into the mold should be done in a quick and rapid movement—a sort of sudden dashing or emptying of a great quantity of metal into the pouring channel and maintaining the pouring channel well filled until the molten metal or alloy rises to the top of the vent channel, as 22. The pouring operation is quite similar to that employed in flushing out a drain with water—a sudden discharge of a considerable quantity of fluid having a head and given a momentum. At the high pouring temperature of the molten brass it is quite fluid and runs rapidly into the mold, but at the same time at this great heat it is giving off tremendous quantities of the gases of volatilization. Referring again to Fig. 1 it will be seen that as the hot metal is dashed into the pouring channel or gate 21 the stream will descend mainly on one side of the vertical tube 26 forcing the heated air and gas within the mold upward on the other side and out through the vent 22, and there will be no conflict between the escaping fluids and the main pouring current. The incoming metal naturally, how-

ever, is splashed about considerably against the parts within the mold and the interior surface the mold itself and great quantities of the gases of volatilization are liberated. 5 These gases, however, being liberated in the unfilled portion of the casting chamber, are instantly free to rise to the vent opening, as 22, and the mold is rapidly filled from the bottom upward with metal which is clear of 10 the gas, and the gas instantly rises through the molten mass and is indeed hastened upward by the solidification of the metal which promptly begins at the bottom of the mold and which is not substantially disturbed 15 by the incoming metal or alloy. While the casting is being made the air and gas are rushing out of the vent in a rapid stream. The opening of the vent into the mold must therefore be of considerable area, 20 and I find in practice that the best results are obtained when this opening is at least substantially the area of the pouring hole where it enters the pouring chamber. In the escape of the heated air and gas the 25 gradually widening walls of the vent channel play an important part, as it is exceedingly important to rid the interior of the mold of the air and gas as rapidly as it can be done. As soon as the gaseous elements 30 pass through the opening 22 of the channel 22 they have opportunity to expand and their expansion continues until they are 35 finally discharged from the mold. As these gaseous elements expand they are naturally projected forward by the tapering walls and the velocity of the gases toward the outside is much greater than if the walls were on parallel lines, the gases thus not only discharging themselves into the air at a 40 high rate of travel, but, it is thought, tending to create a vacuum within the mold so that the remaining gases are sucked toward the discharge opening and their rate of discharge movement considerably accelerated. 45 Another point deemed of importance is now mentioned in that the shrinkage of brass is very great, namely about or fully one-half greater than that of iron. The shrinkage is greater, of course, when the 50 metal is very highly heated. This shrinkage begins as soon as the cast begins to solidify. In the use of chills which have not been sufficiently heated or of such dimensions as to cool rapidly after being heated there is 55 promptly formed a chilled surface upon the casting where it contacts the mold, this chilling in some instances preventing the mold from being entirely filled and, as shown by my previous unsuccessful efforts, the outer 60 surface of the casting becoming set and the interior portion thereof cooling and shrinking, this outer chilled surface is drawn inwardly and is crumpled or buckled, making wrinkle-like irregularities and thus an un- 65 even and defaced piece of work. In the

practice of the art as herein disclosed, however, this difficulty and objection are overcome, for in the provision of a well heated mold and the two large heads of molten metal in the vent and gate channels respectively the shrinkage of the metal within the mold is more uniform and the indications are that the shrinkage in the casting chamber draws still molten metal from the central portions of at least the gate casting, 70 which thus forms a source of supply for the interior shrinkage as indicated. The outer face of the casting is thus preserved smooth and free from the cracks and wrinkles always shown heretofore in the futile attempts to master this art. After solidification has taken place the top surface of the gate casting particularly shows a deep depression, as indicated by the dotted line 35 in Fig. 1. When the gate casting is broken off, the casting again placed within the chill and the gate channel again filled up the amount of shrinkage is indicated by the dotted line 36. 80 85

In Fig. 8 I have shown the application of this art to the formation of an ornamental knob directly upon the end of a tube. In the past brass balls, knobs or other ornaments have been affixed to the ends of rods or tubes, as in bed construction, by means of screws or rivets passing through the walls of a ferrule, sleeve or collar fitting the end of the rod and secured upon the ornament, and sometimes by a stud bolt secured either to the knob or to the tubing and threaded into the other member. All methods heretofore tried for securing such ornaments upon the bed frame have proved not only expensive but very unsatisfactory, and common experience teaches that these knobs are continually working loose or coming off. By the practice of this art these brass heads, or indeed any suitable form of ornament, may be cast directly upon the tube or rod, and once there it would require the use of tools, such as a saw and chisel, to get them off. In casting such a part as the knob 45 I prefer to make the chill or mold substantially as shown in Fig. 8, and the method of making the casting is the same as that already described. The two sections of the mold are provided with complementary casting chamber recesses 41 and complementary trough-like recesses 21 and 22 for the gate and vent channels, substantially as 100 in the chill of Fig. 1. The open mold is shown as containing the end of the rod 44 having a cap 28 as in Fig. 1, the tube being broken away to show a sectional view of the cap. In Fig. 9 the ball or knob 45 is shown 105 as cast upon the rod 44. 110 115 120 125

In Fig. 7 I have shown a bedstead end frame made of metallic rods or tubes 50 secured to a bent metallic rod or tube 51 and a transverse rod or tube 52 by means of 130

connections 40 similar to that shown in Fig. 6. Ornaments 53 of brass may be cast directly upon the rod 51 and the foot ornaments 54 may be similarly applied. A bed frame as illustrated in Fig. 7 would be constructed according to this practice preferably by positioning separate molds upon a work frame in the relation to each other shown by the connections or ornaments in the drawings, placing the metallic parts so that the portions to be connected together are positioned within the molds respectively, the ends of the rods being closed as hereinabove described, the chills having been sufficiently heated beforehand. The assembling of the parts is preferably done with the chill frame in substantially horizontal position, but before the castings are made the frame is swung into vertical position with the mouths of the casting channels upward. The metal is then poured rapidly into the molds, one after the other, until all are filled. The frame may then be lowered into horizontal position, the chills unlocked and opened and the bed frame with the parts and ornaments secured together removed.

An important feature of this art is that the rods and tubes forming the bed frame or other structure may be finished and polished prior to connecting the parts together, and as this finishing and polishing may be done by machinery, it is obvious that a further great advantage results from making the connections in the manner herein set forth. Another exceedingly valuable feature of this art is that the castings come out clear and bright and true to the configuration of the mold. No machining is necessary for most work provided the casting surfaces of the mold are finished smooth. Sometimes it may be desirable to dip the casting momentarily in a solution of one part of commercial sulfuric acid to two parts of water, or it may be desirable to buff certain portions of the casting to bring out high surfaces for the sake of artistic contrast; but the usual dressing, finishing and polishing of the connection or casting are unnecessary, except, of course, that the gate and vent castings must be broken or cut off and the cut surfaces smoothed, which may be done in any well known way. When the parts are taken out of the mold it is found that not only is the casting shrunk tightly upon the metal rods or tubes, but at least in the case of brass rods or tubes the casting is actually sweated upon the parts. This is probably due to the raising of the temperature of the brass rod or tube to the temperature at which the zinc upon or close to the surface of the rod or tube is melted so as to unite with the particles of zinc and copper of the casting alloy. This of course adds greatly to the strength of the connection.

The chills or molds may be conveniently made of gray iron cast in sand and dressed to shape in ways well known to the chill casting art; but cast steel and wrought steel molds milled to shape are naturally more enduring.

While I have illustrated and described certain embodiments of means and have set forth certain steps and conditions in the practice of this new art, it should be understood that this disclosure does not attempt to describe modifications, all within the scope of the discovery and inventions set forth, suitable to adapt the same for use in other manufactures than that of bedstead construction, this particular application of the art being selected merely as an appropriate one for illustrative purposes; and it should further be understood that the particular description of the process as applied to brass casting is intended also merely to illustrate the practice of the art with a common type of volatilizable alloy, brass being appropriately selected because of the extent of use to which this alloy is put and of the numerous attempts to answer the question in the use of brass. Reference should be had therefore to the appended claims, in view of the foregoing description, to determine the scope of the discovery and invention herein specified, and all modifications and changes within the limitations herein set forth are contemplated by me as fall within the scope of these claims.

I claim:

1. The method of casting in a refractory impermeable mold which consists in introducing a volatilizable metal or alloy at a volatilizing temperature into such mold, and freeing the mold of the gases of volatilization during the introduction therein of such metal or alloy.

2. The method of casting in a refractory impermeable mold which consists in introducing a volatilizable metal or alloy at a volatilizing temperature into such mold, and simultaneously relieving the mold of the pressure of the gases of volatilization therein.

3. The method of casting in a refractory impermeable mold which consists in introducing a volatilizable metal or alloy at a volatilizing temperature into such mold at a point substantially on the same horizontal plane as the highest point of the casting chamber of the mold when in casting position, and permitting the free escape from the mold of so much of the gases of volatilization during the casting process as will result in a casting free from blow-holes and similar imperfections.

4. The method of casting in a chill which consists in introducing a volatilizable metal or alloy at a volatilizing temperature into the chill in such manner that the gases of volatilization of the incoming metal may at

100

95

75

80

85

90

95

105

110

115

120

125

130

all times be liberated in the unfilled portion of the casting chamber, and permitting the free escape from such unfilled portion of the casting chamber of the liberated gases of volatilization.

5. The method of casting in a chill which consists in introducing a volatilizable metal or alloy at a volatilizing temperature into the chill in such manner that 10 the gradually upwardly extending solidification of the cooling metal or alloy from the bottom of the casting chamber will not be materially disturbed by the incoming metal or alloy, and permitting the free escape from the chill of the gases of volatilization which are successively liberated from the incoming metal introduced into such chill.

6. The method of casting in a refractory 20 mold of the chill type which consists in heating the mold, heating a volatilizable metal or alloy to a volatilizing temperature, introducing such metal or alloy into the mold in such manner that solidification of 25 the metal may begin at the bottom of the casting chamber and continue upwardly without substantial disturbance by additional incoming metal, and permitting the gases of volatilization to escape from the 30 mold in advance of the rising metal in the casting chamber.

7. The method of securing metallic parts together by means of a cast connection made from metal or alloy which volatilizes 35 with heat, formed *in situ* upon the parts, in impermeable refractory molds, which consists in positioning the parts to be connected within the casting chamber of such mold, introducing a volatilizable metal or 40 alloy at a volatilizing temperature into such mold in such manner that solidification of the molten metal begins substantially at the bottom of the casting chamber and continues upwardly without substantial disturbance 45 by the incoming metal or alloy, and permitting the free escape of the gases of volatilization from the casting chamber in advance of the rising metal or alloy within the casting chamber during the process of 50 casting.

8. The method of casting in a chill mold which consists in initially heating the chill, pouring a volatilizable metal or alloy at a 55 volatilizing temperature into the chill in such manner that the gases of volatilization of the incoming metal may at all times be liberated in the unfilled portion of the mold, and continuously freeing such unfilled portion of the mold of the liberated gases of 60 volatilization by means of forces supplied by the metal or alloy during the casting operation.

9. The method of casting in a refractory 65 impermeable mold of the chill type which consists in introducing a volatilizable metal

or alloy at a volatilizing temperature into such mold, and freeing the mold of the gases of volatilization by utilizing thereto the expansive force of such gases within the mold.

10. The method of casting in a refractory impermeable mold which consists in heating the mold, beating a volatilizable metal or alloy to a volatilizing temperature, introducing the metal or alloy so heated into such mold in such manner that the 75 gases of volatilization may at all times be liberated in the unfilled portion of the mold, and freeing the mold of the gases of volatilization by utilizing thereto the expansive force of such gases of volatilization. 80

11. The method of casting in a refractory impermeable mold which consists in heating a volatilizable metal or alloy to a volatilizing temperature, introducing the metal or alloy so heated into such mold, 85 and freeing the mold of the gases of volatilization by accelerating their discharge through their own expansive force during their escape from the mold.

12. The method of casting in a refractory impermeable mold of the chill type which consists in heating a volatilizable metal or alloy to a volatilizing temperature, pouring the metal or alloy so heated into such mold in such manner that the incoming 90 metal will at no time pass through the metal which has substantially come to rest within the casting chamber of the mold, and freeing the casting chamber of the mold of the gases of volatilization by utilizing 95 their own expansive force thereto.

13. The method of casting in a refractory impermeable mold which consists in heating the mold, beating a volatilizable metal or alloy to a volatilizing temperature, 10 introducing the metal or alloy so heated into the mold at all times above the constantly rising surface of metal or alloy within the mold, and freeing the mold of the gases of volatilization in advance of the 110 rising metal within the mold solely through the expansive force of such volatilizing gases and the force of the constantly rising metal or alloy within the mold.

14. The method of casting in a refractory impermeable mold which consists in introducing a volatilizable metal or alloy at a volatilizing temperature into such mold, and simultaneously relieving the mold of the pressure of the gases of volatilization 120 through the sole action of the expansive force of such gases within the mold and the rising surface of the casting metal within the mold.

15. The method of casting in a refractory 125 impermeable mold which consists in pouring in a quick and rapid movement a volatilizable metal or alloy at a volatilizing temperature into such mold, and simultaneously relieving the mold of the pressure of the 130

gases of volatilization by means of forces operating thereto solely within the mold.

16. The method of casting in a refractory impermeable mold which consists in introducing a volatilizable metal or alloy at a volatilizing temperature into such mold, and relieving the mold of the pressure therein of the gases of volatilization through forces self-contained in the metal or alloy and developed incidentally to its introduction into the mold.

17. The method of casting in a refractory impermeable mold which consists in introducing a volatilizable metal or alloy at a volatilizing temperature into such mold, and simultaneously expelling the gases of volatilization from the mold.

18. The method of casting in a mold of refractory impermeable material which consists in pouring a volatilizable metal or alloy at a volatilizing temperature into such mold in such manner that it descends upon the rising surface of the metal or alloy within the mold, and expelling the gases of volatilization from the mold during the pouring operation.

19. The method of casting in a mold of impermeable material which consists in pouring a volatilizable metal or alloy at a volatilizing temperature into the mold in such manner that it descends upon the continuously rising surface of the metal or alloy within the mold, and expelling the gases of volatilization through an opening in the mold provided for that purpose.

20. The method of casting in a mold of impermeable material which consists in initially heating the mold, heating a volatilizable metal or alloy to a volatilizing temperature, introducing rapidly such metal or alloy into such mold in such manner that it descends substantially on one side thereof, and conducting the gases of volatilization out of said mold.

21. The method of casting in a mold of impermeable material of the chill type which consists in initially heating the mold, introducing a volatilizable metal or alloy at a volatilizing temperature into such mold in such manner that it descends in a rapid stream substantially on one side thereof, and conducting the gases of volatilization out of said mold at a point substantially on another side thereof.

22. The method of casting in a mold of impermeable material which consists in initially heating the mold, pouring a volatilizable metal or alloy at a volatilizing temperature continuously and in a rapidly flowing stream into such mold until the pouring chamber thereof is filled, and expelling the free gases of volatilization from said mold by means of forces solely within the mold during the pouring operation.

22. The method of casting in a refractory

impermeable mold which consists in pouring a volatilizable metal or alloy at a volatilizing temperature into such mold in such manner that the metal being poured acts as a plug to prevent the intake of air into such mold with the poured metal or alloy while it is being poured, and freeing the mold of the gases of volatilization therin.

24. The method of casting in a refractory impermeable mold which consists in rapidly pouring a volatilizable metal or alloy at a highly volatilizable temperature into such mold in such manner that the molten metal enters the casting chamber of such mold under the pressure of a head of molten metal, and freeing the mold of the gases of volatilization during the casting process.

25. The method of casting in a refractory impermeable mold which consists in introducing a volatilizable metal or alloy at a volatilizing temperature into such mold, providing a head of molten metal in communication with the metal entering the casting chamber of the mold, said head of molten metal being so arranged as to supply the interior of the mold with additional metal to prevent injurious contraction of the casting within the mold due to shrinkage, and freeing the mold of the gases of volatilization during the casting operation.

26. The method of casting in a refractory impermeable mold which consists in pouring a volatilizable metal or alloy at a highly volatilizing temperature into such mold in such manner that the molten metal enters the casting chamber of such mold in a rapid and continuous stream and under the pressure of a head of molten metal, which head of molten metal acts as a stop or plug to prevent the intake into the casting chamber of air with the metal being poured, and freeing the mold of the gases of volatilization during the pouring operation by means of forces operating thereto solely within the mold during the pouring operation.

27. The method of casting in a refractory impermeable mold which consists in pouring a volatilizable metal or alloy at a highly volatilizing temperature into such mold in such manner that the molten metal enters the casting chamber of such mold in a rapid and continuous stream and under the pressure of a head of molten metal, and freeing the mold of the gases of volatilization by the sole action of forces within the mold during the pouring operation.

28. The method of casting in a refractory impermeable mold which consists in initially heating the mold, pouring a volatilizable metal or alloy at a highly volatilizing temperature into such mold in such manner that the molten metal enters the casting chamber of such mold in a rapid and continuous stream and under the pressure of

- 5 a head of molten metal, and freeing the mold of the gases of volatilization solely through the action of the expansive force of the gases themselves and the constantly rising surface of the metal within the mold.
- 5 29. The method of casting in a refractory impermeable mold, which consists in initially heating the mold, pouring a volatilizing metal or alloy at a highly volatilizing temperature, into such mold in such manner that the flow of the incoming metal is at no time impeded by congealed or partially congealed metal or alloy within the casting chamber of the mold, and freeing the casting chamber of the mold of the gases of volatilization by its free and unimpeded escape through an opening in a wall of the mold provided for such purpose, and by means of forces operating thereto solely within the mold during the pouring operation.
- 10 30. The process of making a casting from volatilizable metals or alloys in a refractory mold of impermeable material, which consists in melting and heating the metal or alloy to a temperature at which it gives off a gas of volatilization, pouring such metal or alloy rapidly into such mold, and freeing the mold of substantially all of the air and free gas of volatilization during the pouring operation.
- 15 31. The process of making a casting from commercial brass in a refractory mold of impermeable material, which consists in melting and heating the brass to a temperature at which it gives off a gas of volatilization, initially heating the mold, pouring the molten brass rapidly into such mold, and freeing the mold of substantially all of the air and free gas of volatilization during the pouring operation.
- 20 32. The process of securing metallic parts together by means of a cast connection made from one of the commercial brasses and formed *in situ* upon the parts in a refractory mold of impermeable material, which consists in heating the mold, heating such brass to a molten condition and to a temperature at which a gas of volatilization is freely given off, positioning within the casting chamber of such mold the parts so to be connected, pouring such brass so heated rapidly into such mold, and expelling substantially all of the air and free gases of volatilization from the mold during the process of casting.
- 25 33. The process of securing metallic parts together by means of a cast connection of yellow brass formed *in situ* upon the parts in an iron mold, which consists in heating the mold, heating the brass to a highly volatilizing temperature, positioning within such mold the parts so to be connected, pouring rapidly into such mold the molten brass so heated, and freeing the mold of substantially all of the air and free gas of volatilization from the mold during the process of casting.
- 30 34. The process of making a casting in a refractory mold of impermeable material from a volatilizable metal or alloy, which consists in heating such mold, reducing the volatilizable metal or alloy to a highly molten state and to a temperature at which a gas of volatilization is freely liberated therefrom, pouring such volatilizing metal or alloy so heated rapidly into the mold, and simultaneously freeing the casting chamber of the mold of substantially all of the free air and gas or gases of volatilization during the process of casting.
- 35 35. The process of making castings from the commercial brasses in a metallic mold of the chill type, which consists in heating the mold, melting the brass and raising the temperature thereof to a highly volatilizing heat, pouring the molten brass so heated rapidly into the casting chamber of the mold, and simultaneously freeing said casting chamber of substantially all of the air and other gases therein during the process of casting.
- 40 36. The process of making a metallic bedstead frame, which consists in arranging the separate parts of the frame in their desired relations to each other and with the portions thereof to be connected extending into metallic molds, heating a volatilizable metal or alloy to a molten state and to a temperature at which a gas of volatilization is given off, pouring such volatilizing metal or alloy rapidly into the molds, and freeing such molds during the casting process of substantially all of the air and free gas of volatilization.
- 45 37. The process of making a metallic bedstead frame which consists in arranging a plurality of refractory molds of impermeable material in predetermined relations to each other, heating such molds, positioning the separate parts of the bedstead frame in their desired relations to each other and with the portions thereof to be connected extending into said molds, heating one of the commercial brasses to a highly molten state and to a temperature at which it freely liberates a gas of volatilization, pouring rapidly such brass so heated into said molds, and freeing the molds of substantially all of the free gas or gases of volatilization and air during the process of casting therein respectively.
- 50 38. The process of making a metallic bedstead frame, which consists in arranging a plurality of refractory molds of impermeable material in predetermined relations to each other, heating such molds, positioning the separate parts of the bedstead frame in their desired relations to each other and with the portions thereof to be connected extend-

ing into said molds, heating brass to a molten state and to a temperature at which it freely liberates a gas, pouring rapidly such so heated brass into said molds, and 5 permitting the escape from said molds respectively of substantially all of the gas or gases of volatilization and air during the process of casting therein.

39. The method of casting volatilizable 10 metals or alloys in a chill which consists in rapidly pouring such metal or alloy at a volatilizing temperature into the chill, and expelling the gases of volatilization therefrom in a single stream from a point at all 15 times above the constantly rising surface of the metal or alloy within the chill.

40. The method of casting volatilizable 20 metals or alloys in a chill which consists in pouring such metal or alloy at a volatilizing temperature into the chill in such manner that solidification thereof may take place beginning at the bottom of the casting chamber and extend upward without substantial disturbance by additional incoming 25 metal or alloy, and expelling the gases of volatilization from the casting chamber in a single stream from a point at all times above the surface of the constantly rising metal or alloy.

30 41. The method of casting volatilizable

metals or alloys in a chill, which consists in initially heating the chill, rapidly pouring such metal or alloy at a volatilizing temperature into the chill in such manner that solidification thereof may take place beginning 35 at the bottom of the casting chamber and extend upward without substantial disturbance by additional incoming metal or alloy, and expelling the gases of volatilization from the chill in such manner that there is 40 at all times a continuous discharging movement in one general direction of the gases within the casting chamber.

42. The method of casting volatilizable 45 metals or alloys in a chill which consists in rapidly pouring such metal or alloy at a volatilizing temperature into the chill in such manner that solidification thereof may take place beginning at the bottom of the casting chamber and extend upward with- 50 out substantial disturbance by additional incoming metal or alloy and expelling the gases of volatilization from the chill in such manner that counter currents of discharging gases will not be formed within the casting 55 chamber during the casting process.

WILLIAM D. HALL.

Witnesses:

FRANKLIN M. WARDEN,  
M. M. KRIESAND.